# EUROPEAN PATENT SPECIFICATION

(11) **EP 1 505 184 B1**
(45) Date of publication and mention of the grant of the patent: **12.01.2011**
(21) Application number: 04254668.9
(22) Date of filing: 04.08.2004
(51) Int. Cl.: D04B 1/02, D04B 21/02, D06M 17/10

(54) **Controlled air permeability composite fabric articles having enhanced surface durability**
Aus Kompositstoff mit kontrolierter Luftdurchlässigkeit hergestellte Waren mit verbesserter Oberflächenhaltbarkeit
Articles d'étoffe composite à perméabilité d'air controlée présentant une meilleure durabilité de surface

(30) Priority: 07.08.2003 US 493275 P
(43) Date of publication of application: 09.02.2005
(73) Proprietor: MMI-IPCO, LLC, Lawrence, MA 01842 (US)
(72) Inventor: Rock, Moshe, Brookline, MA 02446 (US); Lumb, Douglas, Atkinson, NH 03811 (US); Haryslak, Charles, Marlborough, MA 01752 (US); Vainer, Gadalia, Melrose, MA 02176 (US)
(74) Representative: Murray, Elisabeth Anne

(56) References cited:
- EP-A- 0 515 206
- EP-A- 0 969 130
- CH-A- 612 818
- DE-A- 3 043 433
- DE-A- 3 533 535
- GB-A- 1 420 497
- US-A- 2 962 384

## Description

### TECHNICAL FIELD

The invention relates to composite fabric articles, and more particularly to composite fabric articles having improved surface durability, in particular without substantial adverse affect on desirable qualities of the fabric, e.g. such as drapability, moisture vapor transport (MVT), hand tactile, etc.

### BACKGROUND

Fabric articles, such as jackets and other outer wear, with qualities desired for use during exercise or exertion, especially warmth and breathability, may be formed, e.g., by circular knit plaited construction or circular knit reverse plaited construction, may be formed with a relatively smooth outer surface (the "technical face") and an inner surface (the "technical back") that can be raised, e.g. by processes such as napping, brushing, sanding, etc., to form an insulating layer of fleece. Unfortunately, in both knit constructions, the durability of the smooth technical face is inferior to many woven constructions, limiting their use in articles intended for harsher outdoor sports. In particular, the fuzziness of the smooth technical face will often have an inferior aesthetic look, as well as poor technical features. The smooth face also tends to fuzz out as the surface picks up snow, which it will not shed easily, to fuzz out during rock climbing, and to fuzz out in specific areas of a garment, e.g. at the elbows or at the shoulders, under the straps of a backpack.

Composite fabric articles are achieved by joining at least one material to a fabric body to attain desirable properties that cannot be attained by the fabric body alone. Laminar composites, for example, having multiple layers joined by an adhesive are sometimes employed to increase the thermal resistance of a fabric body. However, the feel (e.g., drapability, hand tactile, etc.) is often substantially decreased by laminating one or more additional layers of material to the fabric body.

EP0515206 describes a composite textile fabric having a first fabric layer whose surface has been raised, and a second fabric layer which may be treated with a polyurethane to promote resistance to pilling.

### SUMMARY

According to one aspect of the invention, a fabric article with knitted or woven construction of multi-filament, interlaced yarns has an inner surface and an outer surface, the inner surface having at least one region of pile or raised fibers or fleece formed thereupon and the outer surface has at least one region of a non-continuous coating of binder material adhered to yarn fibers and at interlacing intersections of yarns, for enhanced durability of the outer surface against pilling or fraying during use as an exposed outer surface of an article of wearing apparel.

Preferred embodiments of this aspect of the invention may include one or more of the following additional features. The fabric article has a plaited circular knit construction, reverse plaited circular knit construction, woven construction or warp knit construction. The fabric article is an article of wearing apparel. The multi-filament yarns are textured or flat. The multi-filament yarns comprise fibers formed of materials selected from the group consisting of: polyester, nylon and polypropylene. The multi-filament yarns of the outer surface comprise spandex. Fibers of the multi-filament yarns are highly intermingled at over about 60 tucks per meter (TPM) and preferably at over about 100 TPM or more, or there may be little or no intermingling. The binder material adheres only to yarn fibers in a manner to substantially avoid restriction of air permeability through the fabric article. Alternatively, the binder material comprises a film extending into interstitial air passageways through the fabric article in a manner to reduce air permeability. The non-continuous coating of binder material is without substantial adverse effect on drapability and hand of the fabric article. The fabric article has one or more first regions of enhanced surface durability due to relatively greater density of binder or binder dots per unit area applied by engineered pattern printing technology to a fabric web. Preferably the one or more first regions comprise shoulder regions. The fabric article has one or more second regions of relatively lesser surface durability due to relatively lesser density of binder or binder dots per unit area applied by engineered pattern printing technology to a fabric web. Preferably, the one or more second regions comprise body regions.

According to another aspect of the invention, a method of forming a fabric article comprises the steps of: interlacing yarns comprising multi-filament fibers to form a fabric body of knit or woven construction, forming a raised or fleece region upon an inner surface of the fabric body; and, thereafter, applying a binder material to at least the outer surface to form a discontinuous coating of binder material upon yarn fibers and at interlacing intersection of yarns on at least the outer surface of the fabric article, to resist pilling and fraying of yarn fibers at the outer surface during use as an exposed outer surface of an article of wearing apparel.

Preferred embodiments of this aspect of the invention may include one or more of the following additional features. The step of applying a binder material comprises applying by standard printing technology, e.g. by rotary screen roll or by gravure roll. The step of applying a binder material comprises applying the binder material with a pad. The method further comprises removing binder material in liquid state from interstitial spaces of the fabric body in a manner to control reduction of air permeability. The step of removing binder material comprises blowing air through the interstitial spaces or drawing air by suction through the interstitial spaces. The step of applying binder material comprises applying a binder material comprising a binder selected from the group consisting of acrylic, polyurethane, silicon and blends thereof, preferably in a form selected from the group consisting of resin, latex, polymer emulsion and polymer dispersion. The step of applying binder material comprises applying a binder material in a liquid carrier and allowing the liquid carrier to evaporate leaving the binder material or applying a binder material in a foam liquid carrier and allowing the foam carrier to collapse leaving the binder material. The step of applying the binder material comprises applying a binder material by engineered pattern printing technology to a fabric web. Preferably, the binder material is applied by engineered pattern printing techniques to form one or more first regions of enhanced surface durability by applying a first pattern with relatively greater density of binder or binder dots per unit area, e.g. to shoulder regions, and to form one or more second other regions of lesser surface durability by applying a second pattern with relatively lesser density of binder or binder dots per unit area, e.g. to body regions.

The invention thus provides a composite fabric article that overcomes the recognized deficiencies of fabrics of knit construction, discussed above, in particular when used in garments and other articles for harsher outdoor sports, without detracting significantly from qualities of the original form of the fabric found highly desirable for use during exercise or exertion, e.g., warmth, breathability, drapability, MVT, hand tactile, etc. Furthermore, improved fabric articles have a predetermined, controlled, i.e., limited, degree of air permeability may be formed according to the method of the invention.

The details of one or more embodiments of the invention are set forth in the accompanying drawings and the description below. Other features, objects, and advantages of the invention will be apparent from the description and drawings, and from the claims.

### DESCRIPTION OF DRAWINGS

FIG 1 is a somewhat diagrammatic view of an example of a fabric article, here, a jacket, of the invention, with an insulating layer of fleece on one or more regions of the inner surface and a non-continuous coating of binder material on one or more regions of the outer surface, for enhanced surface durability.
FIG 2 is a somewhat diagrammatic plan view of the outer surface of a fabric article of the invention, with the binder material for enhanced surface durability against fraying and pilling adhered to yarns and yarns fibers about an interstitial space; and
FIG 3 is a somewhat diagrammatic plan view of the outer surface of a fabric article of the invention, with the binder material for enhanced surface durability against fraying and pilling adhered to yarns and yarns fibers and also extending into interstitial spaces to increase wind resistance.
FIG 4 is a plan view of a fabric web printed with a series of predetermined patterns of binder material applied by engineered pattern printing technology to form regions of enhanced surface durability; and
FIG. 5 is a plan view of a garment, here, a shirt, formed with elements cut from the fabric web of FIG 4 and having enhanced surface durability regions at the shoulders.

Like reference symbols in the various drawings indicate like elements.

### DETAILED DESCRIPTION

Referring to FIG 1, a fabric article of wearing apparel 8, in this case, by way of example only, a jacket, is formed of an improved composite fabric 10 of the invention. The fabric has an inner surface 12, upon which is formed at least one insulating region fleece 14, and an outer surface 16, upon which is adhered a discontinuous coating 18 of binder or coagulant material, e.g. resin or latex, for enhanced surface durability, e.g. against pilling and fraying. Referring also to FIG 2, in a preferred embodiment, regions 20 of binder or coagulant material are adhered primarily to yarn fibers 22 and at interlacing intersections of yarns 24, thereby allowing the fabric to retain its original form and characteristics, including good drapability and hand, and allowing through-passage of air to a predetermined degree (MVT and breathability), but also providing an outer surface of enhanced durability, e.g. against pilling and wear, e.g. during exercise and harsher outdoor sports.

Referring to FIG 3, in other embodiments, as described more fully below, the binder material forms a film 26 that constricts (but preferably does not block) interstitial spaces 28 between yarns 22, thereby to reduce air-permeability and provide increased insulation and warmth, for use in particular under colder and windier conditions.

In a first example of a fabric article to be provided with an outer surface of enhanced durability according to the invention, the fabric has a plaited circular knit construction, e.g., as described in Knitting Technology, by David J. Spencer (Woodhead Publishing Limited, 2nd edition, 1996), with a smooth outer surface (technical face) and a raised inner surface (technical back). The stitch yarn forming the technical face is preferably a filament yarn of textured filaments formed of synthetic material, e.g. polyester, nylon or polypropylene, the yarn fibers or filaments having a high level of intermingling, e.g. at least over about 60 tucks per meter, and preferably over about 100 tucks per meter, to reduce the tendency of individual fibers to fray or catch and later on to pill. In preferred embodiments, the yarn has a fineness of 0.2 to 3.0 denier per filament (dpf); fraying is a particular concern in multi-fiber yarns, especially with yarns of fine dpf, e.g. 0.2 to 1.5.

In a second example of a fabric article to be provided with the outer surface of enhanced durability, the fabric has a reverse plaited circular knit construction, where the raised surface can be formed on the loop yarn, either on the loop side (technical back), which is preferred, or on the smooth side (technical face). The technical back can be any of a variety of constructions, e.g., knit and/or knit-tuck and/or knit-welt and/or knit-tuck-welt in a variety of combinations.

To avoid restricting or reducing the capability of maximizing the bulk of the raised or fleece surface at the technical back, the fabric articles of knit construction are preferably finished before application of the binder material to the outer surface.

In yet another example, the fabric has a woven construction of synthetic, multi-filament, textured yarn. Spandex is incorporated into the yarn, e.g. in air tuck, cover or core spun position, to provide the fabric with two-way or one-way stretch.

In still another example, the fabric upon which a surface of enhanced durability is to be formed has a warp knit construction, e.g. as described in my earlier U.S. Patent Nos. 6,196,032, issued March 6, 2001, and 6,199,410, issued March 13, 2001, .

A fabric article, e.g. from the examples described above, is next treated to provide an outer surface of enhanced durability by applying binder material to reduce fiber fraying and minimize pilling.

In a preferred embodiment, a chemical binder material for forming a surface region of enhanced durability surface is applied to the smooth outer surface of the fabric article using standard printing technology, e.g. rotary or gravure roll. The binder is preferably applied in a non-continuous coating, e.g. a pattern of separate dots. Any suitable chemical binder material may be employed. Examples of such binders include resin (such melamine), latex (such as acrylate), polymer emulsions or dispersions (such as silicon), or polyurethane. The binder is preferably selected to have a dry hand upon curing or drying, i.e. not tacky to the touch, good stretch/recovery, and good bond to textile fibers.

In another preferred embodiment, referring to FIGS. 4 and 5, a suitable binder material for forming a region of enhanced surface durability is applied by engineered pattern printing technology to a fabric web 30 (FIG 4). For example, in FIG 5, a shirt 40, formed with elements cut from fabric web 30, has surface regions 42, 44 of enhanced durability at the shoulders, which are more prone to abrasion and wear when carrying a backpack. Other regions of the shirt 40, e.g., the body region 46, may also be printed to provide enhanced surface durability. However, regions of less wear, e.g. such as the body region 46, may be printed in a different pattern with relatively less density of binder or binder dots per unit area.

Referring again to FIG 4, the predetermined pattern of binder material is applied to the fabric web 30 in a series of shirt piece patterns 32, 32', 32" of predetermined configuration, using engineered pattern printing technology. In a later cut and sew process (not shown), the printed fabric web 30 is indexed through a cutter where shirt pieces are cut from the web and then subsequently sewn together in shirts 40.

In another embodiment, the binder for forming a surface region of enhanced durability surface is applied to the outer surface of the fabric article with a pad. In this embodiment, in order to reduce the tendency toward fraying while maintaining a high level of moisture vapor transmission, good drapability, hand and soft touch, deposit of the binder material is preferably limited primarily to the fibers and/or to the intersections of fibers in the yarn segments, and formation of binder film in the interstitial spaces between yarns is minimized. The formation of film may particularly be avoided by removal of excess liquid binder from interstitial spaces between yarns shortly following application, e.g. while the binder material is still wet or moist, by air suction or air blowing through the fabric article.

Preferably, the binder material is applied in a low viscosity system, or in a system with a relatively low level of binder solids or particulates in a liquid carrier, so that as the system dries, the liquid carrier evaporates (or in a foam system, collapses), leaving the solid binder deposited primarily or only on the yarns or yarn fibers. In this manner, the air permeability level and other characteristics of the base fabric are maintained.

In other embodiments, a binder material of relatively higher viscosity may be employed, to encourage formation of a fine film in the interstitial areas between yarns that will partially or fully maintain its integrity during the drying process. In this manner, the fabric article may be provided with increased water repellency and wind resistance, which would be advantageous in cold windy ambient environments. However, a full or continuous film is typically to be avoided, in order to maintain at least a minimum desired degree of moisture vapor transmission necessary for comfort during high energy activities, such as running, skiing, etc.

Referring again to FIG 1, the garment 8 formed of the fabric article 10 of this embodiment of the invention thus has an outer surface 16 with a non-continuous binder coating 18 providing weather protection, with high pill resistance, high abrasion resistance, and pick resistance, and an inner surface 12 with a raised insulating region 14 with high bulk and softness. In particular embodiments, the fabric article may be provided with water repellence and wind protection.

The improved surface durability of fabric articles of the invention is demonstrated in a severe pitting and abrasion test, such as the modified Martindale abrasion test method of ASTM D 4966. According to this test method, a fabric article of the invention to be tested is subjected to repeated rubbing by a strip of the hook element (General Application type, ¾-inch by ½-inch) of a hook-and-loop type fastener element. After 250 rubs, the appearance of the fabric article of the invention has been seen to be markedly better, e.g., as compared to untreated fabric articles.

A number of embodiments of the invention have been described. Nevertheless, it will be understood that various modifications may be made.

For example, other aesthetic effects may be applied face side to back side, including, e.g., color differentiation and/or patterning on one or both surfaces, including three dimensional effects. As mentioned above, the fabric article may have one-way or two-way stretch, and/or the fabric may be constructed to provide a degree of stretch from any of a broad range, including from very low stretch (very stable) or high stretch or compression power stretch. The binder material may be applied in other fashions as appropriate, e.g. by kiss coating or froth foam application, preferably to the technical face after raising the technical back. In other applications, the binder material may also be deposited, e.g., by pad application, upon both surfaces of the fabric article, including, e.g., upon a raised or fleece surface. The multi- strand or multi-filament yarn may, e.g., have the form of staple fibers in spun yarn or filaments in continuous yarn, or the fabric may be constructed with a combination of spun yarn, staple fibers and continuous filament yarn. In addition to suction and blowing of air through the fabric article during drying, the degree of film formation may also be controlled, e.g., by crushing the coated fabric between nip rollers.

Also, referring again to FIGS. 4 and 5, in other embodiments, only selected regions, e.g., shoulders 42, 44 may be printed to provide enhanced surface durability, and other regions of the shirt 40, e.g. the body region 46, may be left untreated to be raised while printed regions 42, 44 remain flat, resisting the napping process.

Accordingly, other embodiments are within the scope of the following claims.

## Claims

1. A fabric article of knitted or woven construction of multi-filament, interlaced yarns, the fabric article having an inner surface (2) and an outer surface (16), the inner surface (12) having at least one region of pile or raised fibers or fleece (14) formed thereupon, and the outer surface having at least one region (20) of a non-continuous coating (18) of binder material adhered to yarn fibers (22) and at interlacing intersections of yarns (24), for durability of the outer surface (16) against pilling or fraying during use as an exposed outer surface of an article of wearing apparel (8).

2. The fabric article of claim 1, wherein the fabric article has a plaited circular knit construction.

3. The fabric article of claim 1, wherein the fabric article has a reverse plaited circular knit construction.

4. The fabric article of claim 1, wherein the fabric article has a woven construction.

5. The fabric article of claim 1, wherein the fabric article has a warp knit construction.

6. The fabric article of claim 1 in the form of an article of wearing apparel (8).

7. The fabric article of claim 1, wherein the multi-filament yarns (22) are textured.

8. The fabric article of claim 1, wherein the multi-filament yarns (22) are flat.

9. The fabric article of claim 1, wherein the multi-filament yarns (22) comprises fibers formed of materials selected from the group consisting of: polyester, nylon and polypropylene.

10. The fabric article of claim 1, wherein the multi-filament yarns (22) of the outer surface (16) comprise spandex.

11. The fabric article of claim 1, wherein fibers of the multi-filament yarns (22) are highly intermingled at over about 60 tucks per meter.

12. The fabric article of claim 11, wherein fibers of the multi-filament yarns (22) are highly intermingled at over about 100 tucks per meter.

13. The fabric article of claim 1 wherein fibers of the multi-filament yarns (22) have little or no intermingling.

14. The fabric article of claim 1, wherein the binder material adheres only to yarn fibers in a manner to substantially avoid restriction of air permeability through the fabric article.

15. The fabric article of claim 1, wherein the binder material comprises a film extending into interstitial air passageways (28) through the fabric article in a manner to reduce air permeability.

16. The fabric article of claim 1, wherein the non-continuous coating (18) of binder material is without substantial adverse effect on drapability and hand of the fabric article.

17. The fabric article of claim 1, wherein the fabric article (40) has one or more first regions (42, 44) of enhanced surface durability due to relatively greater density of binder or binder dots per unit area applied by engineered pattern printing technology to a fabric web (30).

18. The fabric article of claim 17, wherein said one or more first regions (42, 44) comprises shoulder regions.

19. The fabric article of claim 1 or claim 17, wherein the fabric article has one or more second regions (46) of relatively lesser surface durability due to relatively lesser density of binder or binder dots per unit area applied by engineered pattern printing technology to a fabric web.

20. The fabric article of claim 19, wherein said one or more second regions (46) comprises body regions.

21. A method of forming a fabric article, said method comprising the steps of:
interlacing yarns comprising multi-filament fibers to form a fabric body of knit or woven construction,
forming a raised or fleece (14) region upon an inner surface (12) of the fabric body; and, thereafter,
applying a binder material to at least the outer surface (16) to form a discontinuous coating (18) of binder material upon yarn fibers and at interlacing intersections of yarns on at least the outer surface of the fabric article, to resist pilling and fraying of yarn fibers at the outer surface during use as an exposed outer surface of an article of wearing apparel.

22. The method of claim 21, wherein the step of applying a binder material comprises applying by standard printing technology.

23. The method of claim 22, wherein the standard printing technology comprises printing by rotary screen roll.

24. The method of claim 22, wherein the standard printing technology comprises printing by gravure roll.

25. The method of claim 21, wherein the step of applying a binder material comprises applying the binder material with a pad.

26. The method of claim 21, further comprising removing binder material in liquid state from interstitial spaces (28) of the fabric body in a manner to control reduction of air permeability.

27. The method of claim 26, wherein the step of removing binder material comprises blowing air through the interstitial spaces (28).

28. The method of claim 26, wherein the step of removing binder material comprises drawing air by suction through the interstitial spaces (28).

29. The method of claim 21, wherein the step of applying binder material comprises applying a binder material comprising a binder selected from the group consisting of acrylic, polyurethane and silicon.

30. The method of claim 29, wherein the binder is in a form selected from the group consisting of resin, latex, polymer emulsion and polymer dispersion.

31. The method of claim 21, wherein the step of applying binder material comprises applying a binder material in a liquid carrier and allowing the liquid carrier to evaporate leaving the binder material.

32. The method of claim 21, wherein the step of applying binder material comprises applying a binder material in a foam liquid carrier and allowing the foam carrier to collapse leaving the binder material.

33. The method of claim 21, wherein the fabric article is formed of a knit construction with a technical face defining the outer surface (16) and a technical back defining the inner surface (12), and the method comprising raising the technical back and thereafter applying the binder material to the technical face.

34. The method of claim 21, wherein the step of applying the binder material comprises applying a binder material by engineered pattern printing technology to a fabric web (30).

35. The method of claim 34, wherein the step of applying the binder material by engineered pattern printing technology to a fabric web (30) comprises:
forming one or more first regions (42, 44) of enhanced surface durability by applying a first pattern with relatively greater density of binder or binder dots per unit area, and
forming one or more second other regions (46) of lesser surface durability by applying a second pattern with relatively lesser density of binder or binder dots per unit area.

36. The method of claim 35, wherein the step of forming one or more regions (42, 44) of enhanced surface durability comprises applying the first pattern with relatively greater density of binder or binder dots per unit area at least upon the shoulder regions.

37. The method of claim 35 or claim 36, wherein the step of forming one or more regions (46) of lesser surface durability comprises applying the second pattern with relatively lesser density of binder or binder dots per unit area at least upon the body regions.

## Patentansprüche

1. Gewebeartikel mit gestrickter oder gewebter Konstruktion aus verflochtenen Multifilamentgarnen, wobei der Gewebeartikel eine innere Oberfläche (2) und eine äußere Oberfläche (16) aufweist, wobei auf der inneren Oberfläche (12) mindestens ein Bereich aus Florfasern oder aufgerauten Fasern oder Flausch (14) ausgebildet ist und die äußere Oberfläche mindestens einen Bereich (20) einer nicht durchgängigen Beschichtung (18) aus Bindematerial aufweist, das an Garnfasern (22) und an Verflechtungsschnittpunkten von Garnen (24) haftet und der Beständigkeit der äußeren Oberfläche (16) gegenüber Knötchenbildung oder Ausfransen dient, während sie als freiliegende äußere Oberfläche eines Bekleidungsartikels (8) verwendet wird.

2. Gewebeartikel nach Anspruch 1, wobei der Gewebeartikel eine plattierte Rundstrickkonstruktion aufweist.

3. Gewebeartikel nach Anspruch 1, wobei der Gewebeartikel eine wendeplattierte Rundstrickkonstruktion aufweist.

4. Gewebeartikel nach Anspruch 1, wobei der Gewebeartikel eine gewebte Konstruktion aufweist.

5. Gewebeartikel nach Anspruch 1, wobei der Gewebeartikel eine Kettengewirkkonstruktion aufweist.

6. Gewebeartikel nach Anspruch 1 in Form eines Bekleidungsartikels (8).

7. Gewebeartikel nach Anspruch 1, wobei die Multifilamentgarne (22) texturiert sind.

8. Gewebeartikel nach Anspruch 1, wobei die Multifilamentgarne (22) eben sind.

9. Gewebeartikel nach Anspruch 1, wobei die Multifilamentgarne (22) Fasern umfassen, die aus Materialien gebildet sind, die aus der Gruppe ausgewählt sind, die aus Folgendem besteht: Polyester, Nylon und Polypropylen.

10. Gewebeartikel nach Anspruch 1, wobei die Multifilamentgarne (22) der äußeren Oberfläche (16) Spandex umfassen.

11. Gewebeartikel nach Anspruch 1, wobei die Fasern der Multifilamentgarne (22) mit über etwa 60 Fängen pro Meter stark verwirbelt sind.

12. Gewebeartikel nach Anspruch 11, wobei die Fasern der Multifilamentgarne (22) mit über etwa 100 Fängen pro Meter stark verwirbelt sind.

13. Gewebeartikel nach Anspruch 1, wobei die Fasern der Multifilamentgarne (22) wenig oder keine Verwirbelung aufweisen.

14. Gewebeartikel nach Anspruch 1, wobei das Bindematerial nur an Garnfasern in der Weise haftet, dass die Einschränkung der Luftdurchlässigkeit durch den Gewebeartikel im Wesentlichen vermieden ist.

15. Gewebeartikel nach Anspruch 1, wobei das Bindematerial einen Film umfasst, der sich in Zwischenraumluftdurchgänge (28) durch den Gewebeartikel in einer Weise erstreckt, dass die Luftdurchlässigkeit verringert ist.

16. Gewebeartikel nach Anspruch 1, wobei die nicht durchgängige Beschichtung (18) von Bindematerial ohne wesentliche nachteilige Wirkung auf die Drapierbarkeit und Griffigkeit des Gewebeartikels ist.

17. Gewebeartikel nach Anspruch 1, wobei der Gewebeartikel (40) einen oder mehrere erste Bereiche (42, 44) mit verbesserter Oberflächenbeständigkeit aufgrund einer relativ größeren Dichte von Bindemittel oder Bindemittelpunkten pro Einheitsfläche aufweist, die durch eine technische Musterdrucktechnologie auf eine Gewebebahn (30) aufgebracht werden.

18. Gewebeartikel nach Anspruch 17, wobei der eine oder die mehreren ersten Bereiche (42, 44) Schulterbereiche umfassen.

19. Gewebeartikel nach Anspruch 1 oder Anspruch 17, wobei der Gewebeartikel einen oder mehrere zweite Bereiche (46) mit relativ geringerer Oberflächenbeständigkeit aufgrund einer relativ geringeren Dichte von Bindemittel oder Bindemittelpunkten pro Einheitsfläche aufweist, die durch eine technische Musterdrucktechnologie auf eine Gewebebahn aufgebracht werden.

20. Gewebeartikel nach Anspruch 19, wobei der eine oder die mehreren zweiten Bereiche (46) Körperbereiche umfassen.

21. Verfahren zum Ausbilden eines Gewebeartikels, wobei das Verfahren die folgenden Schritte umfasst:
Verflechten von Garnen mit Multifilamentfasern, um einen Gewebekörper mit gestrickter oder gewebter Konstruktion zu bilden;
Ausbilden eines aufgerauten Bereichs oder Flauschbereichs (14) auf einer inneren Oberfläche (12) des Gewebekörpers; und danach
Aufbringen eines Bindematerials zumindest auf die äußere Oberfläche (16), um eine diskontinuierliche Beschichtung (18) von Bindematerial auf Garnfasern und an Verflechtungsschnittpunkten von Garnen zumindest auf der äußeren Oberfläche des Gewebeartikels zu bilden, um eine Beständigkeit gegenüber Knötchenbildung und Ausfransen von Garnfasern an der äußeren Oberfläche zu schaffen, während sie als freiliegende äußere Oberfläche eines Bekleidungsartikels verwendet wird.

22. Verfahren nach Anspruch 21, wobei der Schritt des Aufbringens eines Bindematerials das Aufbringen durch eine Standarddrucktechnologie umfasst.

23. Verfahren nach Anspruch 22, wobei die Standarddrucktechnologie das Drucken durch eine Rundschablonenwalze umfasst.

24. Verfahren nach Anspruch 22, wobei die Standarddrucktechnologie das Drucken durch eine Tiefdruckwalze umfasst.

25. Verfahren nach Anspruch 21, wobei der Schritt des Aufbringens eines Bindematerials das Aufbringen des Bindematerials mit einem Tampon umfasst.

26. Verfahren nach Anspruch 21, das ferner das Entfernen von Bindematerial im flüssigen Zustand aus den Zwischenräumen (28) des Gewebekörpers in der Weise, dass die Verringerung der Luftdurchlässigkeit gesteuert wird, umfasst.

27. Verfahren nach Anspruch 26, wobei der Schritt des Entfernens von Bindematerial das Blasen von Luft durch die Zwischenräume (28) umfasst.

28. Verfahren nach Anspruch 26, wobei der Schritt des Entfernens von Bindematerial das Saugen von Luft durch einen Sog durch die Zwischenräume (28) umfasst.

29. Verfahren nach Anspruch 21, wobei der Schritt des Aufbringens von Bindematerial das Aufbringen eines Bindematerials mit einem Bindemittel, das aus der Gruppe ausgewählt ist, die aus Acryl, Polyurethan und Silicium besteht, umfasst.

30. Verfahren nach Anspruch 29, wobei ein Bindemittel in einer Form vorliegt, die aus der Gruppe ausgewählt ist, die aus Harz, Latex, Polymeremulsion und Polymerdispersion besteht.

31. Verfahren nach Anspruch 21, wobei der Schritt des Aufbringens von Bindematerial das Aufbringen eines Bindematerials in einem flüssigen Träger und das Ermöglichen, dass der flüssige Träger verdampft, wobei das Bindematerial belassen wird, umfasst.

32. Verfahren nach Anspruch 21, wobei der Schritt des Aufbringens von Bindematerial das Aufbringen eines Bindematerials in einem flüssigen Schaumträger und das Ermöglichen, dass der Schaumträger zusammenfällt, wobei das Bindematerial belassen wird, umfasst.

33. Verfahren nach Anspruch 21, wobei der Gewebeartikel aus einer Strickkonstruktion mit einer technischen Vorderseite, die die äußere Oberfläche (16) definiert, und einer technischen Rückseite, die die innere Oberfläche (12) definiert, ausgebildet wird, und das Verfahren das Aufrauen der technischen Rückseite und anschließend das Aufbringen des Bindematerials auf die technische Vorderseite umfasst.

34. Verfahren nach Anspruch 21, wobei der Schritt des Aufbringens des Bindematerials das Aufbringen eines Bindematerials durch eine technische Musterdrucktechnologie auf eine Gewebebahn (30) umfasst.

35. Verfahren nach Anspruch 34, wobei der Schritt des Aufbringens des Bindematerials durch eine technische Musterdrucktechnologie auf eine Gewebebahn (30) umfasst:
Ausbilden von einem oder mehreren ersten Bereichen (42, 44) mit verbesserter Oberflächenbeständigkeit durch Aufbringen eines ersten Musters mit relativ größerer Dichte von Bindemittel oder Bindemittelpunkten pro Einheitsfläche, und
Ausbilden von einem oder mehreren zweiten anderen Bereichen (46) mit geringerer Oberflächenbeständigkeit durch Aufbringen eines zweiten Musters mit relativ geringerer Dichte von Bindemittel oder Bindemittelpunkten pro Einheitsfläche.

36. Verfahren nach Anspruch 35, wobei der Schritt des Ausbildens von einem oder mehreren Bereichen (42, 44) mit verbesserter Oberflächenbeständigkeit das Aufbringen des ersten Musters mit relativ größerer Dichte von Bindemittel oder Bindemittelpunkten pro Einheitsfläche zumindest auf die Schulterbereiche umfasst.

37. Verfahren nach Anspruch 35 oder Anspruch 36, wobei der Schritt des Ausbildens von einem oder mehreren Bereichen (46) mit geringerer Oberflächenbeständigkeit das Aufbringen des zweiten Musters mit relativ geringerer Dichte von Bindemittel oder Bindemittelpunkten pro Einheitsfläche zumindest auf die Körperbereiche umfasst.

## Revendications

1. Article d'étoffe ayant une structure tricotée ou tissée de fils multifilament entrelacés, l'article d'étoffe ayant une surface intérieure (12) et une surface extérieure (16), au moins une région de fibres bouclées ou grattées ou de molleton (14) étant formée sur la surface intérieure (12), et la surface extérieure ayant au moins une région (20) d'enduction discontinue (18) de liant collé aux fibres à filer (22) et aux intersections d'entrelacement des fils (24), pour garantir la durabilité de la surface extérieure (16) contre le boulochage ou l'effilochage durant l'utilisation comme surface extérieure exposée d'un article de vêtement (8).

2. Article d'étoffe selon la revendication 1, dans lequel l'article d'étoffe a une structure de tricot circulaire tressé.

3. Article d'étoffe selon la revendication 1, dans lequel l'article d'étoffe a une structure de tricot circulaire tressé inversée.

4. Article d'étoffe selon la revendication 1, dans lequel l'article d'étoffe a une structure tissée.

5. Article d'étoffe selon la revendication 1, dans lequel l'article d'étoffe a une structure à mailles jetées.

6. Article d'étoffe selon la revendication 1, ayant la forme d'un article de vêtement (8).

7. Article d'étoffe selon la revendication 1, dans lequel les fils multifilament (22) sont texturés.

8. Article d'étoffe selon la revendication 1, dans lequel les fils multifilament (22) sont plats.

9. Article d'étoffe selon la revendication 1, dans lequel les fils multifilament (22) comprennent des fibres formées de matériaux sélectionnés dans le groupe composé de : polyester, nylon et polypropylène.

10. Article d'étoffe selon la revendication 1, dans lequel les fils multifilament (22) de la surface extérieure (16) comprennent du spandex.

11. Article d'étoffe selon la revendication 1, dans lequel les fibres des fils multifilament (22) sont fortement entremêlées à plus de 60 nervures par mètre environ.

12. Article d'étoffe selon la revendication 11, dans lequel les fibres des fils multifilament (22) sont fortement entremêlées à plus de 100 nervures par mètre environ.

13. Article d'étoffe selon la revendication 1, dans lequel les fibres des fils multifilament (22) sont peu ou pas entremêlées.

14. Article d'étoffe selon la revendication 1, dans lequel le liant adhère uniquement aux fibres de fil de façon à éviter sensiblement une limitation de la perméabilité à l'air de l'article d'étoffe.

15. Article d'étoffe selon la revendication 1, dans lequel le liant comprend un film s'étendant dans des passages d'air interstitiels (28) traversant l'article d'étoffe de façon à réduire la perméabilité à l'air.

16. Article d'étoffe selon la revendication 1, dans lequel l'enduction discontinue (18) de liant n'a aucun effet néfaste sensible sur l'aptitude au drapement et le toucher de l'article d'étoffe.

17. Article d'étoffe selon la revendication 1, dans lequel l'article d'étoffe (40) a une ou plusieurs premières régions (42, 44) présentant une durabilité de surface améliorée en raison d'une densité relativement plus grande de liant ou de points de liant par unité de surface appliqués au moyen d'une technologie spécifique d'impression de dessins sur une bande de tissu (30).

18. Article d'étoffe selon la revendication 17, dans lequel lesdites une ou plusieurs premières régions (42, 44) comprennent des régions d'épaule.

19. Article d'étoffe selon la revendication 1 ou la revendication 17, dans lequel l'article d'étoffe a une ou plusieurs deuxièmes régions (46) présentant une durabilité de surface sensiblement inférieure en raison d'une densité relativement moins grande de liant ou de points de liant par unité de surface appliqués au moyen d'une technologie spécifique d'impression de dessins sur une bande de tissu.

20. Article d'étoffe selon la revendication 19, dans lequel lesdites une ou plusieurs deuxièmes régions (46) comprennent des régions de corps.

21. Procédé pour former un article d'étoffe, ledit procédé comprenant les étapes consistant à :
entrelacer des fils comprenant des fibres multifilament pour former un corps d'étoffe ayant une structure tricotée ou tissée,
former une région grattée ou molletonnée (14) sur la surface intérieure (12) du corps d'étoffe ; puis
appliquer un liant sur au moins la surface extérieure (16) pour former une enduction discontinue (18) de liant sur les fibres à filer et aux intersections d'entrelacement des fils sur au moins la surface extérieure de l'article d'étoffe,
pour empêcher le boulochage ou l'effilochage des fibres à filer sur la surface extérieure durant l'utilisation comme surface extérieure exposée d'un article de vêtement.

22. Procédé selon la revendication 21, dans lequel l'étape consistant à appliquer un liant comprend l'application au moyen d'une technologie classique d'impression.

23. Procédé selon la revendication 22, dans lequel la technologie classique d'impression comprend l'impression par cadre rotatif.

24. Procédé selon la revendication 22, dans lequel la technologie classique d'impression comprend l'impression par rouleau gravé.

25. Procédé selon la revendication 21, dans lequel l'étape consistant à appliquer un liant comprend l'application du liant au moyen d'un tampon.

26. Procédé selon la revendication 21, comprenant en outre l'enlèvement du liant à l'état liquide des espaces interstitiels (28) du corps d'étoffe de manière à contrôler une réduction de la perméabilité à l'air.

27. Procédé selon la revendication 26, dans lequel l'étape consistant à enlever le liant comprend le soufflage d'un air à travers les espaces interstitiels (28).

28. Procédé selon la revendication 26, dans lequel l'étape consistant à enlever le liant comprend la circulation d'un air par aspiration à travers les espaces interstitiels (28).

29. Procédé selon la revendication 21, dans lequel l'étape consistant à appliquer un liant comprend l'application d'un liant comprenant un liant sélectionné dans le groupe composé d'acrylique, de polyuréthanne et de silicium.

30. Procédé selon la revendication 29, dans lequel le liant se présente sous une forme sélectionnée dans le groupe composé de résine, de latex, d'émulsion de polymère et de dispersion de polymère.

31. Procédé selon la revendication 21, dans lequel l'étape consistant à appliquer un liant comprend l'application d'un liant dans un véhiculeur liquide et le fait de permettre au véhiculeur liquide de s'évaporer pour quitter le liant.

32. Procédé selon la revendication 21, dans lequel l'étape consistant à appliquer un liant comprend l'application d'un liant dans un véhiculeur liquide moussant et le fait de permettre au véhiculeur moussant de s'affaisser pour quitter le liant.

33. Procédé selon la revendication 21, dans lequel l'article d'étoffe est formé d'une structure tricotée avec une face technique définissant la surface extérieure (16) et un dos technique définissant la surface intérieure (12), le procédé comprenant le lainage du dos technique, puis l'application du liant sur la face technique.

34. Procédé selon la revendication 21, dans lequel l'étape consistant à appliquer le liant comprend l'application d'un liant au moyen d'une technologie spécifique d'impression de dessins sur une bande de tissu (30).

35. Procédé selon la revendication 34, dans lequel l'étape consistant à appliquer le liant au moyen d'une technologie spécifique d'impression de dessins sur une bande de tissu (30) comprend :
la formation d'une ou plusieurs premières régions (42, 44) présentant une durabilité de surface améliorée en appliquant un premier dessin ayant une densité relativement plus grande de liant ou de points de liant par unité de surface, et
la formation d'une ou plusieurs deuxièmes régions (46) présentant une durabilité de surface inférieure en appliquant un deuxième dessin ayant une densité relativement moins grande de liant ou de points de liant par unité de surface.

36. Procédé selon la revendication 35, dans lequel l'étape consistant à former une ou plusieurs régions (42, 44) présentant une durabilité de surface améliorée comprend l'application du premier dessin ayant une densité relativement plus grande de liant ou de points de liant par unité de surface sur des régions d'épaule.

37. Procédé selon la revendication 35 ou la revendication 36, dans lequel l'étape consistant à former une ou plusieurs régions (46) présentant une durabilité de surface inférieure comprend l'application du deuxième dessin ayant une densité relativement moins grande de liant ou de points de liant par unité de surface sur des régions de corps.
